# EUROPEAN PATENT APPLICATION

(11) **EP 4 524 278 A1**
(43) Date of publication of application: **19.03.2025**
(21) Application number: 23826544.1
(22) Date of filing: 21.06.2023
(51) Int. Cl.: C22C 38/00, C22C 38/58, C21D 8/02

(54) **HIGH REAMING STEEL AND MANUFACTURING METHOD THEREFOR**

(30) Priority: 22.06.2022 CN 202210714666; 22.06.2022 CN 202210714629
(71) Applicant: Baoshan Iron & Steel Co., Ltd., Shanghai 201900 (CN)
(72) Inventor: WANG, Huanrong, Shanghai 201900 (CN); ZHANG, Chen, Shanghai 201900 (CN); YANG, Ana, Shanghai 201900 (CN); PANG, Houjun, Shanghai 201900 (CN); FAN, Jiajie, Shanghai 201900 (CN)
(74) Representative: Maiwald GmbH
(86) International application number: PCT/CN2023/101836
(87) International publication number: WO 2023/246899

(57) **Abstract**

The present invention provides a steel and a method for manufacturing therefor. The steel comprises the following components in the percentage by mass: C: 0.01-0.10%; Si: ≤0.2%; Mn: 0.5-2.0%; P: ≤0.02%; S: ≤0.003%; Al: 0.01-0.08%; N: ≤0.004%; V: 0.10-0.50%; O: ≤0.003%; and the balance of Fe and inevitable impurities. The steel of the present invention can be applied in passenger vehicle chassis parts needing high strength and thickness reduction such as a control arm and a subframe.

## Description

### TECHNICAL FIELD

The present invention relates to a steel and a method for manufacturing therefor, in particular to a high hole expansion steel and a method for manufacturing therefor.

### BACKGROUND

Vehicle plays a very important role in the development of national economy. Many parts in passenger vehicle, especially some parts of the chassis and body, often require hot-rolled pickled products. Lightweight of passenger vehicle is a development trend in the automotive industry. The high strength and weight reduction of vehicles require higher grades of steel, and the structure of the chassis also needs to be improved, resulting in more complex chassis parts and higher requirements for material properties, surface conditions, and forming technologies, such as hydroforming, hot stamping, laser welding, etc., thus transforming into performance requirements for materials such as high strength, stamping, flanging, rebound and fatigue performance.

At present, the high hole expansion steel used by domestic vehicle parts companies is basically high-strength steel with a tensile strength of 600MPa or less. There is considerable competition for high hole expansion steel with a tensile strength of 540MPa or less. At the same time, high hole expansion steel with a tensile strength of 780MPa is gradually being used in batches in China. However, the elongation and hole expansion ratio, two important indicators in the forming process, are also demanding, while the requirements for performance stability are becoming more stringent.

In order to reduce process costs, passenger vehicle companies have further improved the performance requirements of the materials. For example, when producing vehicle chassis parts, in order to reduce the steps of the stamping process, the material is required to have high strength and high plasticity as well as a high hole expansion ratio. For example, the hole expansion ratio of 780MPa grade high hole expansion steel is required to be guaranteed to be ≥50%, preferably further increase to 70% or even 80% or more. Existing high hole expansion steel, especially 780MPa grade high hole expansion steel, mostly have hot-rolled bainite structures and are strengthened with precipitated phases at the same time. Most of the process paths used are medium-temperature coiling, but the temperature control accuracy is not high and the uniformity of finished product structure is poor, resulting in ununiform properties, such as hole expansion ratio, of the obtained hot-rolled steel, and stamping cracking is prone to occur during subsequent processing.

Prior arts of 780 MPa grade pickled high hole expansion steel are listed below:
Chinese patent CN103602895A discloses a low carbon Nb-Ti micro-alloyed high hole expansion steel, which adopts a composition design of low carbon, high silicon in combination with Nb-Ti micro-alloying, which can ensure a hole expansion ratio of ≥50%. However, the design of high silicon composition usually results in red scale on the surface of the steel plate. In addition, the coiling temperature required to form bainite is usually around 500°C, which makes it difficult to control the temperature on full length of the steel coil, resulting in large fluctuations in the performance of the entire length of the steel coil.

Chinese patent CN105821301A discloses an 800MPa grade hot-rolled high-strength high hole expansion steel, which also adopts a composition design of low carbon and high silicon in combination with Nb-Ti micro-alloying. The Ti content in the steel is very high, ranging from 0.15 to 0.18%. In the actual production process, this composition design will lead to defects such as red scale on the surface of the strip steel. On the other hand, due to the high Ti content, coarse TiN is easily formed in the steel, which is detrimental to the stability of the hole expansion ratio.

Chinese patent CN108570604A discloses a 780MPa grade hot-rolled pickled high hole expansion steel, which adopts a composition design of low carbon, high aluminum and high chromium, and adopts a three-stage cooling process in the process design. Although there is no red scale on the surface of the strip steel, the high aluminum composition design can easily cause clogging of the casting nozzle during the actual production process. On the other hand, the production process of this steel is complex, especially the three-stage cooling process is difficult to control, resulting in a low hole expansion ratio of the steel.

Chinese patent CN114107792A discloses a 780MPa grade hot-rolled pickled high hole expansion steel, which adopts a composition design of low carbon and high titanium and an appropriate amount of molybdenum is added to the steel. Since the phase transformation process of molybdenum-containing steel is relatively slow, the phase transformation process mainly occurs after coiling. Therefore, in the actual production process, there are problems such as low strength of the inner and outer rings of steel coils.

### SUMMARY

In view of the above-mentioned defects in the prior arts, an objective of the present invention is to provide a steel and a method for manufacturing therefor. The steel of the present invention has high strength, high plasticity and high hole expansion ratio, and these properties are well-matched with each other, and can be used in passenger vehicle chassis parts needing high strength and thickness reduction such as a control arm and a subframe.

To achieve the above objective, the present invention adopts the following technical solution:
In order to meet user demands for the matching of higher surface quality, better performance stability, plasticity and hole expansion property, conventional high hole expansion steel needs to be improved.

**In** general, the elongation of a material is inversely proportional to the hole expansion ratio, that is, the higher the elongation, the lower the hole expansion ratio; conversely, the lower the elongation, the higher the hole expansion ratio. Under the same or similar strengthening mechanism, the higher the strength of the material, the lower the hole expansion ratio. **In** order to obtain steel with both good plasticity and hole expansion flanging performance, a better balance between the two is needed. **In** order to achieve a good matching between strength, plasticity and hole expansion performance, the addition of higher amounts of silicon elements seems to be indispensable for high-strength high-plasticity high hole expansion steel. However, the compositional design of high silicon usually leads to poor surface quality of steel plates. Specifically, the red scale defects formed during the hot rolling process are difficult to be completely removed in the subsequent pickling process, resulting in appearance of stripe-shaped red scale on the surface of the pickled high-strength steel, which seriously affects the surface quality.

The present invention optimizes the chemical composition of the existing hot-rolled steel by adopting a low carbon and high vanadium element design without intentionally adding silicon element to the steel, and by adding the V element to improve the strength and plasticity of the steel by taking advantage of the nano-sized vanadium carbide it forms. A bainitic precipitation-strengthened high-strength steel with uniform structure and properties can be obtained without changing the existing hot continuous rolling production line.

Specifically, the steel according to the present invention comprises the following components in percentage by mass: C: 0.01-0.10%; Si≤0.2%; Mn: 0.5-2.0%; P≤0.02%; S≤0.003%; Al: 0.01-0.08%; N≤0.004%; V: 0.10-0.50%; O≤0.003%; and the balance of Fe and inevitable impurities.

Preferably, the steel further comprises Ti, with an upper limit of 0.2%, preferably 0.18%, more preferably 0.015%, and a lower limit of 0.05%, preferably 0.08% in percentage by mass.

Preferably, the steel further comprises 0.1-0.5%, more preferably 0.20-0.40%, still more preferably 0.2-0.3% of Mo in percentage by mass.

Preferably, the steel further comprises one or more components selected from Nb≤0.1%, Cu≤0.5%, Ni≤0.5%, Cr≤0.5%, and B≤0.002%, wherein Cu is more preferably 0.3% or less; Ni is more preferably 0.3% or less; Cr is more preferably 0.3% or less; Nb is more preferably 0.06% or less; B is more preferably 0.002% or less, still more preferably 0.001% or less.

Preferably, the composition of the steel satisfies one or more of the following: C: 0.03-0.07%; Si≤0.10%; Mn: 0.8-1.6%; S≤0.0018%; Al: 0.02-0.05%; N≤0.003%; O≤0.002%.

In the composition design of the steel according to the present invention:
Ca is a basic element in steel and one of the important elements in the present invention. C can expand the austenite phase area and stabilize the austenite. As an interstitial atom in steel, C plays a very important role in improving the strength of steel, among which it has the greatest impact on the yield strength and tensile strength of steel. In the present invention, since the structure to be obtained during the hot rolling stage is low carbon bainite, in order to obtain high hole expansion steel with final tensile strength reaching different strength levels, the C content must be 0.01% or more; at the same time, the C content must not be higher than 0.10%. If the C content is too high, low carbon martensite is easily formed during low-temperature coiling. Therefore, the present invention controls the C content to 0.01-0.10%, preferably 0.03-0.07%.

Si is a basic element in steel. As mentioned before, in order to meet user demands for high strength, high plasticity and high hole expansion ratio, a higher amount of Si is usually added in the composition design. However, the composition design of high silicon brings about a reduction in the surface quality of the steel plate, which has higher amount of red scale defects. In the present invention, in order to ensure good surface quality, the Si content should be strictly controlled during component design. In other words, Si is an impurity element in the present invention. Considering that Si-Mn is needed for deoxidation in actual steelmaking, it seems difficult to completely avoid the addition of Si. According to a large amount of statistical data from actual production, when the Si content is 0.2% or less, the surface red scale defects can be avoided during the hot rolling process. Usually, when the Si content is 0.10% or less, it is guaranteed that no red scale will appear. Therefore, the Si content in the steel of the present invention is controlled within 0.2%, preferably within 0.10%.

Mn is also the most basic element in steel and one of the most important elements in the present invention. It is well known that Mn is an important element in expanding the austenite phase area. It can reduce the critical quenching speed of steel, stabilize austenite, refine grains, and postpone the transformation of austenite to pearlite. In the present invention, in order to ensure the strength and grain refinement effect of the steel plate, the Mn content is usually controlled at 0.5% or more; at the same time, the Mn content should not generally exceed 2.0%, otherwise Mn segregation will easily occur during steelmaking, and hot cracking is also prone to occur during continuous casting of slabs. Therefore, the Mn content in the steel of the present invention is controlled at 0.5-2.0%, preferably 0.8-1.6%.

P is an impurity element in steel. P is very easy to segregate on the grain boundaries. When the P content in the steel is high (≥0.1%), Fe₂P will be formed and precipitated around the grains, reducing the plasticity and toughness of steel. Therefore, the lower its content, the better. The present invention controls the P content within 0.02%, and the steel obtained has better mechanical performances and does not increase the cost of steelmaking.

S is an impurity element in steel. S in steel usually combines with Mn to form MnS inclusions. Especially when the contents of S and Mn are both high, more MnS will be formed in the steel. MnS itself has a certain plasticity, it would deform along the rolling direction during the subsequent rolling process, which not only reduces the transverse plasticity of the steel, but also increases the anisotropy of the structure, which is detrimental to the hole expansion performance. In order to reduce the MnS content, the S content needs to be strictly controlled. The lower the S content in the steel, the better. In the present invention, the S content is controlled within 0.003%, preferably 0.0018% or less.

Al's main function in steel is to deoxidize and fix nitrogen. In the presence of strong carbide-forming elements such as Ti, the main function of Al is to deoxidize and refine grains. In the present invention, Al is a common deoxidizing element and grain refining element, and its content is usually controlled at 0.01-0.08%; when the Al content is less than 0.01%, it will not have the effect of refining grains; similarly, when the Al content is higher than 0.08%, its effect of refining grains will reach saturation. Therefore, the Al content in the steel of the present invention is controlled between 0.01-0.08%, preferably between 0.02-0.05%.

N is an impurity element in the present invention, and the lower its content, the better. However, N is an inevitable element in the steelmaking process. Although its content is low, in combination with strong carbide forming elements such as V, the VN particles formed adversely affect the performance of the steel, especially very detrimental to the hole expansion performance. Due to the square shape of VN, there is a large stress concentration between its sharp corners and the substrate. During the process of hole expansion deformation, the stress concentration between VN and the substrate can easily form crack sources, thus greatly reducing the hole expansion performance of the material. Since the present invention adopts a high vanadium design in the composition system, in order to minimize the adverse effect on hole expansion caused by VN, the present invention controls the N content to 0.004% or less, preferably 0.003% or less.

V is an important element in the present invention. Similar to Ti and Nb, V is also a strong carbide-forming element. However, vanadium carbides have low solid-solution or precipitation temperature and are usually fully solid-solutionized in austenite during the finishing rolling stage. Only when the temperature is lowered and phase transformation begins, V begins to form in the ferrite. In order to fully utilize the precipitation strengthening effect of V, the amount of V added to the steel should be at least 0.10% or more to have obvious precipitation strengthening effect; as the V content increases, the precipitation strengthening effect of V gradually increases. When the V content exceeds 0.50 %, the precipitation strengthening effect of V is saturated and the size of the vanadium carbide formed is larger, which adversely reduces the contribution to the steel strength. Therefore, the amount of V added to the steel of the present invention is controlled to be ≤0.50%. Specifically, when the V content is 0.10-0.20%, a 590MPa grade high hole expansion steel can be obtained; when the V content is 0.20-0.35%, a 780MPa grade high hole expansion steel can be obtained; when the V content is 0.35 -0.50%, a 980MPa grade high hole expansion steel can be obtained.

Mo is one of the important elements in the present invention. The addition of Mo in steel can greatly postpone the phase transformation of ferrite and pearlite, which is conducive to obtaining a bainite structure. In addition, Mo has strong resistance to welding softening. Since the main objective of the present invention is to obtain a low carbon bainite structure, and low carbon bainite is prone to softening after welding, adding a certain amount of Mo can effectively reduce the degree of welding softening. Therefore, in the present invention, the Mo content is controlled at 0.10-0.50%, preferably 0.20-0.40%, more preferably 0.2-0.3%. When combined with the sectional cooling process, Mo plays a certain inhibiting role in the formation of ferrite during the sectional cooling process. When the Mo content is within the above range, its effect can be fully realized.

Nb is one of the addable elements in the present invention. Nb, similar to Ti, is a strong carbide element in steel. The addition of Nb in steel can greatly increase the non-recrystallization temperature of the steel, obtain deformed austenite with higher dislocation density during the finishing rolling stage, and refine the final phase change structure during the subsequent transformation process. However, the amount of Nb added should not be too much. On one hand, if the amount of Nb added exceeds 0.10%, it is easy to form relatively coarse niobium carbonitrides in the structure, consuming part of the carbon atoms and reducing the precipitation strengthening effect of carbides. At the same time, the higher Nb content also tends to cause anisotropy of the hot-rolled austenite structure, which is inherited to the final structure during the subsequent cooling phase transformation process, harming the hole expansion performance. Therefore, the Nb content in the steel of the present invention is controlled at ≤0.10%, preferably ≤0.06%.

Ti is an optional element in the present invention. The addition of a small amount of Ti in steel can, on one hand, combine with N to form TiN during the high-temperature stage, which can fix N and help reduce the subsequent formation of VN; on the other hand, the excess Ti after combining with N can be combined with C to form nano-TiC during the subsequent process and improve the performance of the steel with the nano-VC together. When the Ti content is higher than 0.20%, coarser TiN is prone to be formed during the high-temperature stage and deteriorates the impact toughness of the steel. Therefore, the content of the optional element Ti in the steel of the present invention is within 0.20%, preferably within 0.18%, more preferably within 0.015%, most preferably within 0.10%. On the other hand, the Ti content is preferably 0.05% or more, more preferably 0.08% or more, which provides an excellent precipitation strengthening effect.

Cu is an optional element in the present invention. The addition of Cu in steel can improve the corrosion resistance of steel. When it is added together with the P element, the corrosion resistance performance is better; when the amount of Cu added exceeds 1%, under certain conditions, an ε-Cu precipitated phase can be formed, causing a strong precipitation strengthening effect. However, the addition of Cu can easily cause the "Cu brittleness" phenomenon during the rolling process. In order to make full use of Cu's corrosion resistance improvement effect in certain applications without causing significant "Cu brittleness" phenomenon, the present invention controls the Cu content to within 0.5%, preferably within 0.3%.

Ni is an optional element in the present invention. The addition of Ni in steel has a certain degree of corrosion resistance, but the corrosion resistance effect is weaker than that of Cu. The addition of Ni in steel has little effect on the tensile performance of the steel, but can refine the structure and precipitated phases of the steel, greatly improving the low-temperature toughness of the steel; at the same time, in steel with added Cu element, adding a small amount of Ni can inhibit the occurrence of "Cu brittleness". Adding a higher amount of Ni has no significant adverse effect on the performance of the steel itself. If Cu and Ni are added at the same time, it can not only improve the corrosion resistance, but also refine the structure and precipitated phases of the steel, greatly improving the low-temperature toughness. However, since both Cu and Ni are relatively expensive alloying elements, in order to minimize the cost of the alloy design, the amount of Ni added to the steel of the present invention is ≤0.5%, preferably≤0.3%.

Cr is an optional element in the present invention. Cr is added to steel to improve the strength of steel mainly through solid solution strengthening or microstructure refinement. Since the structure of the steel in the present invention is fine bainitic ferrite plus nano-precipitated carbides, the ratio of yield strength and tensile strength of the steel, i.e., the yield ratio, is relatively high, and usually reaches 0.90 or more. Adding a small amount of Cr can appropriately reduce the yield strength of steel, thereby reducing the yield ratio. In addition, adding a small amount of Cr can also improve corrosion resistance. Usually, the amount of Cr added is ≤0.5%, preferably ≤0.3%.

B is an optional element in the present invention. B can greatly improve the hardenability of steel, promote bainite transformation, and promote lath bainite transformation during medium-temperature bainite phase transformation. Therefore, adding a trace amount of B to the steel is conducive to obtaining a fine lath bainite structure. However, the B content should not be too much. Adding too much B will lead to the formation of martensite and more M-A islands, which is unfavorable to plasticity and hole expansion. Therefore, the amount of B added in the steel of the present invention is controlled at ≤0.002%, preferably ≤0.001%.

O is an impurity element in the present invention. In order to obtain steel with better performance, the lower the O content in the steel, the better. However, a lower oxidation amount will increase the cost of steelmaking. In order to ensure the performance of the strip steel, the O content in the steel of the present invention is controlled to be within 0.003%, preferably within 0.002%.

Existing high hole expansion steels are usually designed with high titanium composition, in which the main purpose of adding micro-alloying element Ti is to refine the grains, and the addition amount is generally within 0.1%. The present invention adopts a high vanadium composition design, and Ti is present as an optional element in the steel of the present invention. The main purpose of adding V in the present invention is to combine it with C to form dispersively distributed nano-vanadium carbide for precipitation strengthening.

The steel of the present invention obtains a steel having both high tensile strength and hole expansion ratio by including a content of V up to 0.1-0.5%. When the V content in the steel is 0.10-0.20%, the tensile strength of the steel is 590MPa, and the hole expansion ratio is ≥70%, preferably ≥80%; when the V content in the steel is 0.20-0.35%, the tensile strength of the steel is 780MPa, and the hole expansion ratio is ≥50%; when the V content in the steel is 0.35-0.50%, the tensile strength of the steel is 980MPa, and the hole expansion ratio is ≥30%, preferably ≥40%.

Most of the microstructures of existing high hole expansion steels are ferrite or ferrite plus bainite. In order to obtain higher strength, nano-titanium carbide is used for strengthening. When the high hole expansion steel of the present invention does not contain Ti, its microstructure is bainite and nano-vanadium carbide in bainite. Moreover, according to the different V content, high hole expansion steel of different strength grades can be obtained to meet the needs of downstream users for different strength grades of high hole expansion steels. When the steel of the present invention contains Ti, its microstructure is ferrite and bainite, wherein the ferrite contains nano-TiC and the bainite contains nano-VC.

The present invention also provides a method for manufacturing the steel of the present invention, including the following steps:

### 1) Smelting and casting

The above composition is smelted by a converter or an electric furnace, secondary refined by a vacuum furnace, and casted into billets or ingots.

### 2) Reheating of billets or ingots

Heating temperature≥1100°C, preferably 1200°C or more; holding time: 1-2 hours.

### 3) Hot rolling and cooling.

As an embodiment of the method for manufacturing the present invention, preferably, in step 3) of the method for manufacturing the present invention, the initial rolling temperature is 1000-1100°C, and rough rolling of 3-5 passes is carried out under high pressure at 950°C or more to a cumulative deformation of ≥50%, then the intermediate billet is air-cooled or water-cooled to 900-950°C, and finishing rolling of 7 passes is carried out to a cumulative deformation of ≥70%, completing the finishing rolling between 800-900°C, and obtaining a steel strip, thereafter, the steel strip is water-cooled to 400-550°C at a cooling rate of ≥10°C/s and coiled, and slowly cooling to room temperature at a cooling rate of ≤20°C/s, obtaining a hot-rolled steel strip.

As another embodiment of the method for manufacturing the present invention, preferably, in step 3) of the method for manufacturing the present invention, the initial rolling temperature of the hot rolling is 1050-1150°C, and rough rolling of 3-5 passes is carried out under high pressure at 1050°C or more to a cumulative deformation of ≥50%, then an intermediate billet is heated to 950-1000°C, and finishing rolling of 3-7 passes are carried out to a cumulative deformation of ≥70%, and the finishing rolling temperature is 800-950°C, and obtaining a steel strip;
wherein the cooling is staged cooling, and after finishing rolling, the steel strip is water-cooled to 600-750°C at a cooling rate of ≥30°C/s, then after air cooling for 1-10 seconds, the steel strip is cooled to 400-550°C at a cooling rate of ≥10°C/s and coiled, then cooling to room temperature at a cooling rate of ≤20°C/h, obtaining a hot-rolled strip steel.

Preferably, when the steel of the present invention contains Ti, it is carried out using the above-mentioned method including sectional cooling.

In the step 3) above, the initial rolling temperature of hot rolling is 1050-1150°C, and rough rolling of 3-5 passes is carried out under high pressure at 1050°C or more to a cumulative deformation is ≥50%. The main purpose is to refine the austenite grains, and retain more solid solutionized Ti at the same time.

In the rough rolling and finishing rolling stages of step 3), rolling should be completed as quickly as possible to ensure that there is more solid solutionized Ti and V in the austenite. After the high-temperature finishing rolling, the steel strip is first cooled to 600-750°C at a cooling rate of ≥30°C/s, then forming ferrite and nano-TiC inside the ferrite grain at the air-cooling stage. The steel strip is subsequently water-cooled to 400-550°C at a cooling rate of ≥10°C/s to obtain bainite and nano-precipitated VC. Eventually, a microstructure dominated by ferrite and bainite and nano-precipitated TiC and VC inside ferrite and bainite is obtained.

When the steel contains both high titanium and high vanadium, the main purpose of adding more V is to make it combine with C to form dispersively distributed nano-VC for precipitation strengthening. The high titanium and high vanadium compositions together with the sectional cooling process results in the formation of nano-TiC inside the ferrite grains in the ferrite formation region, and nano-VC inside the bainite in the bainite formation region. Through the combination of compositions and processes, the excess Ti after combining with N can be formed with C into nano-TiC in the air-cooling stage after the first water-cooling stage, which serves to strengthen the ferrite. Introducing nano-TiC into ferrite can reduce the performance difference between ferrite and bainite, which is conducive to improve the hole expansion ratio; by controlling the strength of bainite through different V contents, high hole expansion steel of different strength grades can be obtained to meet the needs of downstream users for different strength grades of high hole expansion steels.

Preferably, the method further includes step 4) Pickling, wherein the pickling operating speed of the hot-rolled strip steel is 30-120m/min, the pickling temperature is 75-85°C, the straightening rate is ≤3%, rinsing is carried out at 35-50°C, and the surface drying and oiling are carried out at 120-140°C to obtain pickled high hole expansion steel.

In the method for manufacturing the steel of the present invention:
The invention adopts a medium-temperature coiling process and combines it with an innovative low carbon, high vanadium and low silicon composition design to obtain a high-strength high hole expansion steel with excellent performance stability.

In the medium and low-temperature bainite transformation region, precise control of the coiling temperature ensures uniformity of performance over the entire length of the strip steel. During the medium-temperature coiling process, bainite phase transformation occurs, accompanied by nano-precipitation of V. By quantifying the content of key elements C and V in conjunction with specific coiling, a series of high hole expansion steel products with different strength grades and different hole expansion ratios can be obtained.

While the conventional high titanium high hole expansion steel mostly adopts high-temperature coiling process, the present invention adopts a medium-temperature coiling process. Therefore, during the rough rolling and finishing rolling stages, the rolling pace should be completed as quickly as possible to ensure that more V is solidly dissolved in austenite. After the high-temperature finishing rolling, the strip steel is cooled on-line to the mid-temperature region of 400-550°C at a cooling rate of ≥10°C/s to obtain bainite and nano-precipitation structure.

When steel contains Ti and sectional cooling is used in the manufacturing process, the desired amount of ferrite is formed and nano-titanium carbide are precipitated inside the ferrite grains at the air-cooling stage after the first water-cooling after rolling to improve the ferrite property; in the medium-temperature coiling stage after the second water-cooling, the precipitation of V is adopted to form nano-vanadium carbide in the bainite, which improves the strength of the bainite. Through the composition and process innovations, ferrite strengthened by nano-titanium carbide and bainite structure strengthened by nano-vanadium carbide are obtained. Through different designs of V content, a series of high hole expansion steel products with different strength grades can be obtained, demonstrating the innovation of compositions and processes and the resulting uniqueness of structure and performance. Nano-TiC and VC give ferrite and bainite higher strength and more balanced properties respectively.

In the subsequent pickling process, the inhomogeneity of thermal stress and organizational stress formed within the steel coil during the medium-temperature coiling phase transformation process is fully released during pickling and straightening, which can further improve the structural uniformity. Based on this innovative design of composition and process, the present invention can obtain a series of high-surface hot-rolled pickled high hole expansion steel products with different strength grades, and excellent plasticity, hole expansion performance, and performance stability.

Compared with the prior arts, the advantages or beneficial effects of the present invention are:
Compared with the high silicon composition design used in Chinese patents CN103602895A and CN105821301A, the present invention adopts a silicon-free and high vanadium composition design to avoid the appearance of red scale on the surface of the strip steel and improve the surface quality of pickled high-strength steel.

Compared with Chinese patent CN108570604A, although its Si content is 0.05-0.5%, it is still not guaranteed to completely eliminate red scale defects on the surface of the strip steel. Moreover, the three-stage cooling process is difficult to control and the performance stability is difficult to guarantee. **In** contrast, the present invention adopts multi-path cooling precision control technique, which can ensure the performance uniformity of the strip steel.

The present invention further adopts innovative low carbon, high titanium and high vanadium composition design, combined with innovative sectional cooling and medium-temperature coiling processes, to obtain hot-rolled pickled high hole expansion steels with excellent surface, strength, plasticity and hole expansion performance of different strength grades and good performance stability.

The steel of the present invention has a tensile strength of ≥590-≥980MPa, and a good elongation (transverse A50≥13%-≥18%) and high hole expansion performance (hole expansion ratio≥30%-≥80%) in a thickness of 1.5-6.0mm, showing matching of excellent surface, strength, plasticity and hole expansion performance, and can be applied to the manufacture of vehicle chassis, subframe and other complex parts that require high strength, thickness reduction, hole expansion and flanging, which has a very broad application prospect.

### BRIEF DESCRIPTION OF THE DRAWINGS

Figure 1 is a schematic diagram of the rolling and cooling process for the steel of Examples 1-9 of the present invention;
Figure 2 is a schematic diagram of the rolling and cooling process for the steel of Examples 10-18 of the present invention;
Figure 3 is a schematic diagram of the cooling process after rolling for the steel of Examples 10-18 of the present invention.

### DETAILED DESCRIPTION

The present invention is further described below with reference to the accompanying examples and drawings.

The steel compositions of Examples 1-18 of the present invention are shown in Table 1, and the balance being Fe and inevitable impurities.

The process path of the steels of Examples 1-18 of the present invention is:

### 1) Smelting and casting

The composition shown in Table 1 was smelted by a converter or an electric furnace, secondary refined by a vacuum furnace, and casted into billets or ingots;

### 2) Reheating of billets or ingots

In Examples 1-9, the heating temperature was ≥1100°C and between 1100-1300°C; in Examples 10-18, the heating temperature was 1200°C or more and between 1200-1300°C. The holding time was 1-2 hours.

### 3) Hot rolling and cooling

In Examples 1-9, primary cooling was used. Specifically, the initial rolling temperature was 1000-1100°C, and rough rolling of 3-5 passes was carried out under high pressure at 950°C or more to a cumulative deformation of ≥50%, then the intermediate billet was air-cooled or water-cooled to 900-950°C, and finishing rolling of 7 passes was carried out to a cumulative deformation of ≥70%, completing the finishing rolling between 800-900°C, then the steel strip was water-cooled to 400-550°C at a cooling rate of ≥10°C/s and coiled, and slowly cooled to room temperature at a cooling rate of ≤20°C/s.

### 4) Pickling

The pickling operating speed of the strip steel was 30-140m/min, preferably 30-120m/min, the pickling temperature was 75-85°C, the straightening rate was ≤3%, rinsing was carried out at 35-50°C, and surface drying and oiling were carried out at 120-140°C.

In Examples 10-18, secondary cooling was used in step 3 above. Specifically, the initial rolling temperature of hot rolling was 1050-1150°C, and rough rolling of 3-5 passes was carried out under high pressure at 1050°C or more to a cumulative deformation of ≥50%, then the intermediate billet was heated to 950-1000°C, and finishing rolling of 3-7 passes was carried out to a cumulative deformation of ≥70%, and the finishing rolling temperature was 800-950°C; cooling was staged cooling, and after finishing rolling, the steel strip was water-cooled to 600-750°C at a cooling rate of ≥30°C/s, after air cooling for 1-10 seconds, the steel strip was cooled to 400-550°C at a cooling rate of ≥10°C/s and coiled, and cooled to room temperature at a cooling rate of ≤20°C/h.

Figure 1 illustrates the procedure of the method for manufacturing the present invention. Table 2 shows the manufacturing process parameters of the steel of Examples 1-18 of the present invention. Table 3 shows the performance parameters of the pickled steel of Examples 1-18 of the present invention.

The steel in Comparative Examples 1-3 is selected from CN103602895A, and the steel in Comparative Example 4 is selected from CN114107792A.

As can be seen from Table 1, none of the compositions of Comparative Example 1-4 contain V elements, while the compositions of Comparative Examples 1-3 also contain high silicon. Therefore, from the perspective of the surface quality of the steel plates, the surfaces of the steel plates of Comparative Examples 1-3 inevitably contain red scale, while the examples of the present invention are all designed with silicon-free compositions and have excellent surface quality.

In addition, all of Comparative Examples 1 to 4 only adopted high titanium composition designs, and no V was added to the steel, indicating that they adopted nano-titanium carbide precipitation strengthening; while the Examples of the present invention adopted high vanadium composition designs and used nano-vanadium carbide for strengthening.

As can be seen from Table 3, through quantitative design and precise control of compositions and key process parameters, the present invention can obtain high hole expansion steels of three different strength grades with a yield strength of ≥500-≥800 MPa, a tensile strength of ≥590-≥980 MPa, an elongation (transverse A50) of ≥13-≥18%, and a hole expansion ratio of ≥30-≥80%.

The mechanical performances of the steel in Table 3 were determined as follows:
The yield strength, tensile strength and elongation (transverse A50) of the steel were tested in accordance with GB/T 228.1-2021 "Tensile Test of Metallic Materials Part 1: Room Temperature Test Methods".

The hole expansion ratio of steel was tested in accordance with GB/T 24524-2021 "Metallic Materials, Thin plates and stripes, Hole expansion test methods".

The steel structure of Examples 1-9 is bainite, and the bainite contains nano-VC, wherein the volume fraction of nano-VC in the bainite is approximately 0.005-0.05%, preferably 0.005-0.03%.

The steel structures of Examples 10-18 are ferrite and bainite, wherein the ferrite contains nano-TiC and the bainite contains nano-VC. Specifically, the volume fraction of ferrite in steel is 10-40%, the volume fraction of nano-TiC in ferrite is about 0.005-0.02%, the volume fraction of bainite in steel is 60-90%, and the volume fraction of nano-VC is bainite is approximately 0.005-0.03%.

As can be seen from the above examples, the high hole expansion steel of the present invention has a good match of high strength, high plasticity and high hole expansion ratio, and is particularly suitable for manufacturing parts such as vehicle chassis structures that require high strength, thickness reduction, hole expansion and flanging forming, which has a broad application prospect.

**Table 1 (unit: percentage by mass)**

| | C | Si | Mn | P | S | Al | N | V | O | Mo | Nb | Ti | Cu | Ni | Cr | B |
|---|---|---|---|---|---|---|---|---|---|---|---|---|---|---|---|---|
| Example 1 | 0.02 | 0.05 | 1.74 | 0.018 | 0.0024 | 0.058 | 0.0025 | 0.10 | 0.0022 | 0.5 | - | 0.10 | - | 0.3 | 0.2 | 0.0015 |
| Example 2 | 0.03 | 0.14 | 1.52 | 0.015 | 0.0028 | 0.074 | 0.0024 | 0.15 | 0.0025 | - | 0.04 | - | 0.4 | - | 0.5 | 0.0012 |
| Example 3 | 0.01 | 0.19 | 1.27 | 0.016 | 0.0023 | 0.052 | 0.0030 | 0.20 | 0.0018 | 0.4 | - | 0.08 | 0.3 | 0.1 | - | 0.0006 |
| Example 4 | 0.05 | 0.16 | 1.43 | 0.011 | 0.0030 | 0.023 | 0.0029 | 0.27 | 0.0023 | - | 0.10 | 0.20 | - | 0.5 | 0.1 | - |
| Example 5 | 0.07 | 0.08 | 1.99 | 0.009 | 0.0025 | 0.045 | 0.0038 | 0.20 | 0.0030 | - | 0.06 | 0.16 | 0.2 | 0.3 | - | - |
| Example 6 | 0.06 | 0.12 | 1.84 | 0.014 | 0.0021 | 0.064 | 0.0035 | 0.35 | 0.0014 | 0.1 | - | - | - | 0.1 | - | 0.0010 |
| Example 7 | 0.10 | 0.07 | 0.76 | 0.017 | 0.0026 | 0.011 | 0.0040 | 0.50 | 0.0020 | - | 0.08 | 0.05 | 0.5 | 0.2 | 0.4 | 0.0019 |
| Example 8 | 0.08 | 0.15 | 0.51 | 0.020 | 0.0029 | 0.032 | 0.0037 | 0.36 | 0.0015 | 0.3 | 0.02 | - | 0.1 | 0.4 | 0.3 | - |
| Example 9 | 0.09 | 0.09 | 1.05 | 0.012 | 0.0020 | 0.080 | 0.0028 | 0.44 | 0.0023 | 0.2 | 0.05 | 0.09 | 0.3 | - | - | 0.0009 |
| Example 10 | 0.02 | 0.15 | 0.95 | 0.014 | 0.0013 | 0.061 | 0.0028 | 0.15 | 0.0023 | - | 0.10 | 0.08 | - | 0.2 | - | 0.0007 |
| Example 11 | 0.03 | 0.13 | 0.77 | 0.013 | 0.0027 | 0.042 | 0.0024 | 0.10 | 0.0028 | 0.5 | - | 0.10 | - | - | 0.5 | - |
| Example 12 | 0.01 | 0.09 | 0.53 | 0.008 | 0.0015 | 0.080 | 0.0040 | 0.20 | 0.0029 | - | - | 0.07 | - | - | - | - |
| Example 13 | 0.04 | 0.20 | 1.73 | 0.010 | 0.0030 | 0.025 | 0.0027 | 0.28 | 0.0025 | - | 0.06 | 0.10 | 0.2 | 0.1 | 0.1 | - |
| Example 14 | 0.07 | 0.08 | 1.26 | 0.012 | 0.0018 | 0.056 | 0.0033 | 0.34 | 0.0020 | 0.3 | - | 0.13 | - | - | - | 0.0020 |
| Example 15 | 0.05 | 0.14 | 1.55 | 0.020 | 0.0025 | 0.073 | 0.0039 | 0.21 | 0.0024 | - | - | 0.15 | 0.5 | - | 0.3 | - |
| Example 16 | 0.09 | 0.10 | 1.99 | 0.009 | 0.0027 | 0.011 | 0.0028 | 0.43 | 0.0030 | - | 0.02 | 0.12 | - | - | - | - |
| Example 17 | 0.08 | 0.13 | 1.84 | 0.016 | 0.0020 | 0.034 | 0.0030 | 0.49 | 0.0026 | 0.1 | - | 0.20 | - | 0.4 | 0.2 | - |
| Example 18 | 0.10 | 0.06 | 1.68 | 0.010 | 0.0026 | 0.057 | 0.0035 | 0.35 | 0.0022 | - | 0.05 | 0.17 | - | 0.5 | - | 0.0015 |
| Comparative Example 1 | 0.045 | 1.10 | 1.70 | 0.010 | 0.0009 | 0.057 | 0.0031 | - | - | - | 0.045 | 0.13 | - | - | - | - |
| Comparative Example 2 | 0.050 | 0.85 | 1.90 | 0.011 | 0.0020 | 0.024 | 0.0031 | - | - | - | 0.060 | 0.11 | - | - | - | - |
| Comparative Example 3 | 0.080 | 0.55 | 1.65 | 0.009 | 0.0010 | 0.051 | 0.0045 | - | - | - | 0.024 | 0.15 | - | - | - | - |
| Comparative Example 4 | 0.060 | 0.070 | 1.73 | 0.011 | 0.0024 | 0.063 | 0.0038 | - | 0.0022 | 0.45 | 0.010 | 0.15 | - | - | - | - |

**Table 2**

| | Heating temperatu re °C | Initial rolling temper ature °C | Cumulative deformatio n of rough rolling % | Intermediat e billet temperature °C | Cumulative deformation of finishing rolling % | Finishing rolling temperature °C | Cooling rate after rolling <°C/s) | Final cooling temperatu re (°C) | Air-cooling time (s) | Water-cooling rate °C/s | Coiling temperat ure °C | Cooling rate °C/h |
|---|---|---|---|---|---|---|---|---|---|---|---|---|
| Example 1 | 1130 | 1030 | 71 | 910 | 93.8 | 810 | - | - | - | 35 | 440 | 12 |
| Example 2 | 1100 | 1000 | 80 | 900 | 95.0 | 840 | - | - | - | 50 | 400 | 17 |
| Example 3 | 1120 | 1010 | 60 | 905 | 94.0 | 800 | - | - | - | 10 | 420 | 5 |
| Example 4 | 1180 | 1060 | 75 | 940 | 96.8 | 830 | - | - | - | 60 | 450 | 17 |
| Example 5 | 1140 | 1040 | 65 | 920 | 95.4 | 820 | - | - | - | 40 | 500 | 13 |
| Example 6 | 1160 | 1050 | 83 | 930 | 96.5 | 880 | - | - | - | 70 | 475 | 20 |
| Example 7 | 1260 | 1100 | 50 | 950 | 95.6 | 850 | - | - | - | 20 | 520 | 7 |
| Example 8 | 1230 | 1090 | 62 | 945 | 96.8 | 870 | - | - | - | 45 | 550 | 15 |
| Example 9 | 1200 | 1080 | 70 | 940 | 93.3 | 900 | - | - | - | 25 | 510 | 10 |
| Example 10 | 1250 | 1110 | 72 | 970 | 94.3 | 870 | 48 | 700 | 7 | 25 | 450 | 8 |
| Example 11 | 1260 | 1120 | 63 | 980 | 98.4 | 910 | 30 | 650 | 1 | 70 | 400 | 7 |
| Example 12 | 1200 | 1050 | 80 | 950 | 88.0 | 800 | 45 | 600 | 4 | 12 | 420 | 10 |
| Example 13 | 1230 | 1080 | 60 | 960 | 97.0 | 860 | 50 | 680 | 2 | 54 | 470 | 13 |
| Example 14 | 1290 | 1140 | 75 | 990 | 96.5 | 920 | 35 | 620 | 8 | 60 | 450 | 11 |
| Example 15 | 1240 | 1070 | 58 | 975 | 95.7 | 830 | 67 | 730 | 6 | 38 | 480 | 15 |
| Example 16 | 1300 | 1150 | 70 | 1000 | 95.7 | 950 | 56 | 750 | 3 | 27 | 500 | 14 |
| Example 17 | 1220 | 1060 | 55 | 965 | 97.7 | 900 | 80 | 660 | 5 | 44 | 530 | 17 |
| Example 18 | 1210 | 1050 | 66 | 955 | 93.9 | 850 | 40 | 710 | 10 | 18 | 550 | 20 |

**Table 3**

| | Steel plate thickness, mm | Yield strength, MPa | Tensile strength, MPa | Elongation, % | Hole expansion ratio, % |
|---|---|---|---|---|---|
| Example 1 | 4.5 | 550 | 620 | 22 | 97.4 |
| Example 2 | 2.5 | 576 | 646 | 19 | 103.6 |
| Example 3 | 6.0 | 543 | 633 | 21 | 100.9 |
| Example 4 | 2.0 | 746 | 804 | 19 | 99.2 |
| Example 5 | 4.0 | 770 | 829 | 18 | 87.5 |
| Example 6 | 1.5 | 758 | 815 | 20 | 90.7 |
| Example 7 | 5.5 | 855 | 998 | 16 | 64.5 |
| Example 8 | 3.0 | 864 | 1035 | 14 | 53.1 |
| Example 9 | 5.0 | 912 | 1027 | 15 | 43.3 |
| Example 10 | 4.0 | 564 | 622 | 19.5 | 89.6 |
| Example 11 | 1.5 | 578 | 634 | 20.5 | 93.4 |
| Example 12 | 6.0 | 601 | 657 | 20.0 | 75.8 |
| Example 13 | 3.0 | 685 | 835 | 18.5 | 73.2 |
| Example 14 | 2.2 | 734 | 826 | 18.0 | 55.6 |
| Example 15 | 4.5 | 777 | 808 | 19.0 | 67.9 |
| Example 16 | 3.2 | 836 | 1023 | 13.0 | 52.5 |
| Example 17 | 2.6 | 808 | 1004 | 14.0 | 44.3 |
| Example 18 | 5.2 | 842 | 1037 | 13.5 | 38.9 |
| Comparative Example 1 | 2.9 | 720 | 790 | 19 | 58 |
| Comparative Example 2 | 2.8 | 710 | 820 | 17 | 65 |
| Comparative Example 3 | 4.0 | 750 | 856 | 15 | 50 |
| Comparative Example 4 | 6.0 | 783 | 832 | 19 | 96 |

## Claims

1. A steel, comprising the following components in percentage by mass:
C: 0.01-0.10%; Si≤0.2%; Mn: 0.5-2.0%; P≤0.02%; S≤0.003%; Al: 0.01-0.08%; N≤0.004%; V: 0.10-0.50%; O≤0.003%; and the balance of Fe and inevitable impurities.

2. The steel as claimed in claim 1, **characterized in that**, the steel further comprises 0.05-0.2%, preferably 0.08-0.15%, more preferably 0.08-0.10% of Ti in percentage by mass.

3. The steel as claimed in claim 1 or 2, **characterized in that**, the steel further comprises one or more components selected from Nb≤0.1%, Cu≤0.5%, Ni≤0.5%, Cr≤0.5%, and B≤0.002% in percentage by mass.

4. The steel as claimed in claim 3, **characterized in that**, the steel further comprises 0.1-0.5%, preferably 0.20-0.40%, more preferably 0.2-0.3% of Mo in percentage by mass.

5. The steel as claimed in claim 1 or 2, **characterized in that**, the components of the steel satisfy one or more of the following: C: 0.03-0.07%; Si≤0.10%; Mn: 0.8-1.6%; S≤0.0018%; Al: 0.02-0.05%; N≤0.003%; O≤0.002%.

6. The steel as claimed in claim 3, **characterized in that**, the components of the steel satisfy one or more of the following: Nb≤0.06%, Cu≤0.3%, Ni≤0.3%, Cr≤0.3%, and B≤0.001%.

7. The steel as claimed in claim 1, **characterized in that**, the steel has a structure of bainite and nano-precipitated VC in bainite.

8. The steel as claimed in claim 2, **characterized in that**, the steel has a structure of ferrite and bainite, wherein the ferrite contains nano-TiC and the bainite contains nano-VC.

9. The steel as claimed in any one of claims 1-8, **characterized in that**, the steel has a yield strength of 500MPa or more, a tensile strength of 590MPa or more, preferably 780MPa or more, and a transverse elongation A50 of 14% or more and 30% or less.

10. A method for manufacturing the steel of any one of claims 1-9, including the following steps:
1) Smelting and casting
The composition of any one of claims 1-9 is smelted by a converter or an electric furnace, secondary refined by a vacuum furnace, and casted into billets or ingots;
2) Reheating the billets or ingots
Heating temperature≥1100°C, holding time: 1-2 hours;
3) Hot rolling and cooling.

11. The method as claimed in claim 10, **characterized in that** in step 3), an initial rolling temperature is 1000-1100°C, and rough rolling of 3-5 passes is carried out under high pressure at 950°C or more to a cumulative deformation of ≥50%, then an intermediate billet is air-cooled or water-cooled to 900-950°C, and finishing rolling of 7 passes is carried out to a cumulative deformation of ≥70%, completing the finishing rolling between 800-900°C and obtaining a steel strip, thereafter, the steel strip is water-cooled to 400-550°C at a cooling rate of ≥10°C/s and coiled, then slowly cooling to room temperature at a cooling rate of ≤20°C/s, obtaining a hot-rolled steel strip.

12. The method as claimed in claim 10, **characterized in that** in step 3), the initial rolling temperature of the hot rolling is 1050-1150°C, and rough rolling of 3-5 passes is carried out under high pressure at 1050°C or more to a cumulative deformation of ≥50%, then an intermediate billet is heated to 950-1000°C, and finishing rolling of 3-7 passes are carried out to a cumulative deformation of ≥70%, and the finishing rolling temperature is 800-950°C, obtaining a steel strip;
wherein the cooling is staged cooling, and after finishing rolling, the steel strip is water-cooled to 600-750°C at a cooling rate of ≥30°C/s, then after air cooling for 1-10 seconds, the steel strip is cooled to 400-550°C at a cooling rate of ≥10°C/s and coiled, then cooling to room temperature at a cooling rate of ≤20°C/h, obtaining a hot-rolled strip steel.

13. The method as claimed in claim 11 or 12, **characterized in that**, the method further includes step 4) Pickling, wherein a pickling operating speed of the hot-rolled strip steel is 30-140m/min, preferably 30-120m/min, a pickling temperature is 75-85°C, a straightening rate is ≤3%, rinsing is carried out at 35-50°C, and surface drying and oiling are carried out at 120-140°C.
